

# UNITED STATES PATENT OFFICE.

JAMES McINTOSH, OF NORRISTOWN, PENNSYLVANIA, ASSIGNOR TO DIAMOND STATE FIBRE COMPANY, OF BRIDGEPORT, PENNSYLVANIA, A CORPORATION OF DELAWARE.

## INDURATED PRODUCT.

1,269,292.

Specification of Letters Patent. Patented June 11, 1918.

No Drawing.

Application filed January 26, 1917. Serial No. 144,761.

*To all whom it may concern:*

Be it known that I, JAMES McINTOSH, a citizen of the United States, and a resident of Norristown, Montgomery county, Pennsylvania, have invented an Indurated Product, of which the following is a specification.

One object of my invention is to provide a product particularly adapted for use in the manufacture of so-called noiseless gears, valves and the like, which shall be not only hard, tough and mechanically strong but in addition shall be impervious to oil, water and moisture and a good insulator.

It is further desired to provide a product of the above noted class which shall have as its base a membranous animal substance such as leather or parchment, and which in addition to the qualities inherent to such substances, shall be practically unaffected by oil and water as well as capable of being mechanically worked and polished.

In carrying out my invention I saturate leather with a liquid, such as acetone, which is a solvent of synthetic resins such as those condensation products of phenol and formaldehyde known as condensite and baekelite, and in the case of ordinary tanned leather varying from a quarter to three-eights of an inch in thickness, an immersion of thirty-six hours in this liquid is sufficient. The saturated leather is then placed in condensite, baekelite or other liquid synthetic resin for about twenty-four hours in which time the acetone is displaced by such liquid;—it being noted however that this time as well as that required for the saturation with acetone may be considerably varied without departing from my invention, since it is dependent upon such variable factors as the nature and thickness of the leather as well as on the temperature, etc.

The displacement of the acetone by the

liquid resin may be materially hastened by agitation, by subjecting the liquid to vacuum which removes the acetone and by slightly heating the liquid, say to about 30° C. After the removal of the acetone, the leather, parchment or other animal membrane is dried at a temperature of from 100°–150° C., for a time sufficient to cause the condensite or other synthetic resin to assume its solid form.

The product resulting from the above described process is hard, tough and close-grained, being readily operated on by tools and capable of taking a high polish. It is moreover water and oil proof and is particularly fitted for use in hot, moist situations where it successfully resists disintegration and maintains its good electrical insulating properties.

If desired, after the leather or other animal fiber has been impregnated with the condensite or other synthetic resin, it may be built up in a series of layers to form a structure of any desired dimensions and thereafter be subjected to pressure and heat whereby such layers are caused to adhere at the same time that the synthetic resin becomes solidified. The resultant product, as in the case of a single layer, is homogeneous and capable of being mechanically worked into such structures as gears and valves.

I claim:—

1. As a new article of manufacture an animal membrane impregnated with solidified synthetic resin.
2. As a new article of manufacture, leather impregnated with solidified synthetic resin.
3. As a new article of manufacture, leather impregnated with solidified condensite.

In witness whereof I affix my signature.

JAMES McINTOSH.